

## UNITED STATES PATENT OFFICE

2,586,590

MANUFACTURE OF LUBRICATING OILS  
FROM SHALE OILPaul Woog, Paris, France, assignor to Compagnie  
Française de Raffinage (Societe Anonyme),  
Paris, FranceNo Drawing. Application June 5, 1946, Serial No.  
674,626. In France August 22, 1941Section 1, Public Law 690, August 8, 1946  
Patent expires August 22, 1961

3 Claims. (Cl. 260—671)

## 1

It is known that crude shale-oils contain a mixture of aliphatic, naphthenic and aromatic hydrocarbons which is characterised, in general, by a relatively high proportion of unsaturated hydrocarbons, of the order of 15 to 60% and a relatively low proportion of aromatic hydrocarbons. Furthermore, these oils contain more or less complex phenols, more or less complex nitrogenous bases, sulphuretted compounds, and various other substances in a comparatively low proportion relatively to the previously mentioned ones.

The unsaturated character of crude shale-oils, which is probably due to the cracking that accompanies the distillation of the schist, does not appear to have been sufficiently taken into consideration heretofore. The treatments which have hitherto been carried out on shale-oil are mainly: either distillation, or cracking, followed by refining in order to obtain engine fuels and lubricating oils; the treatments are preceded or accompanied by alkaline and acid washing which is intended to remove the phenols and the bases.

The cracking treatment does not enable gas-oil with a good ketene number, or good quality lubricating oil to be obtained.

The distillation treatment may produce: a comparatively low proportion of heavy spirit, burning oil, gas-oil, distillates for the manufacture of oils, and residues. Owing to the high percentage of unsaturated and to a considerable proportion of aromatic hydrocarbons, the gas-oils obtained have a low ketene number, and the losses in the refining of the distillates for oils are substantial (the unsaturated and the aromatic hydrocarbons being carried away by the ordinary refining agents).

I have discovered that the polymerization and/or the arylation of the unsaturated hydrocarbons enables novel and much more advantageous results to be obtained. For this purpose the oil, according to the cases, being freed or not of the bases and of all or part of the phenols and acids, it is necessary to make the unsaturated hydrocarbons react, either on themselves (by polymerization), or on the aromatic (or even naphthenic) hydrocarbons contained in the oil, or added to the oil. It is also possible to convert the unsaturated hydrocarbons into chemical derivatives which are easy to separate from the mass, as will be explained hereinafter.

In the fraction distilling between the limits of the gas-oil, the extraction of the unsaturated and of the aromatic hydrocarbons by polymerization and/or arylation increases the ketene number, in particular when the percentage of remaining naphthenic hydrocarbons is comparatively low.

## 2

On the other hand, the products of polymerisation or of arylation obtained are lubricating oils of high viscosity and having a viscosity index which is sufficient for practical uses.

5 In the distillates for oil, the extraction of the unsaturated hydrocarbons leaves an oil of which the stability is increased and which can be refined by means of the usual refining agents, with comparatively low losses. Its viscosity index is also increased if the percentage of remaining naphthenic hydrocarbons is small enough. On the other hand, the polymerisation or the arylation products obtained are oils which are much more viscous than the residue.

10 15 The operations of polymerization and/or of arylation can be applied to any other fraction of the shale-oil, and produce viscous oils.

Arylation can also be effected by adding to more or less narrow fractions of shale-oil, from 20 which certain products have been removed as hereinbefore stated, aromatic hydrocarbons such as benzene, toluene, xylene and homologous substances, naphthalene and homologous substances, anthracene, and heavier, synthetic aromatic products, such as diphenyl or dibenzyl and their homologues, or finally synthetic or natural oils 25 which are rich in aromatic nuclei such as those described in French Patent No. P. V. 458,994, filed on June 23, 1941, in the name of Compagnie 30 Francaise de Raffinage.

The results obtained by the treatment of shale-oils claimed by me are characterized by a considerable increase in the yield of viscous oils. On the one hand, the yield by weight is increased by 35 the reduction of the losses in the refining of the oil distillates, in the usual refining operations, by the conversion into oil of unsaturated products belonging not only to the oil distillates, but to all the fractions of the shale-oil, and finally the possibility of adding to the initial shale-oil aromatic products from an external source, and of incorporating them in the finished oil. On the other hand, the lubricating oils obtained by the treatment claimed may be more viscous than 40 those contained in the most viscous distillates of 45 the initial shale-oil.

The products obtained from the first arylation of the olefines with the aromatics and in particular with benzene or naphthalene, can be reacted again with a suitable proportion of dihalo-alkyl. 50 This operation enables the viscosity of the polymers to be increased.

The catalysts used for these polymerisations are those generally considered suitable for the reaction of Friedel and Crafts and in particular the halides of aluminum, of boron or of iron, an-

## 3

timony, tin. Catalysts mainly comprising phosphoric acids may also be used.

The elimination of phenols from the oil need not necessarily be carried out thoroughly. It may be advantageous in order to maintain a high resistance to the oxidation of the oils, either to leave in the oil subjected to reaction, or to incorporate in the polymerization product obtained, a small quantity of the phenols of the original oil. The heavy phenols are recommended for engine oils owing to their comparatively low volatility.

Consequently, it may be recommended for certain shale-oils to fractionate the oil in more or less narrow fractions before reaction and even before dephenolating. The dephenolating need not be carried out thoroughly in the fractions which actually contain phenols which have the desired characteristics and which it is desired to retain in the oil.

On the other hand, the fractionating of shale-oil before polymerization or arylation may produce, with certain shale-oils, by means of the same operations, results which are distinctly better than those which are obtained without prior fractionation, in particular as regards the viscosity index and chiefly when the fractions containing olefines having unbranched or slightly branched chains of 8 to 18 atoms of carbon are comparatively poor in aromatic substances.

It is also possible to effect the polymerization or the arylation operations after fixing halogens or halogen acids on the unsaturated hydrocarbons, or halogens on the saturated hydrocarbons, this latter substitution increasing the yield of oil.

20

25

30

35

**A. Dephenolating.**—The oils are washed 3 times with about 10% of soda. Stir. Decant. Separate the phenolic lye. These alkaline washings are followed by a washing with water.

**B. Polymerization.**—To the dephenolated oil add 10% of anhydrous aluminium chloride and stir for 48 hours at a temperature of 60° C.

**C. Treatment.**—The tars formed are allowed to settle, then the liquid remaining above is decanted. This liquid is washed: (1) with water containing  $\frac{1}{2}$  of hydrochloric acid; (2) with water; (3) with water alkalised with soda.

**D. Distillation.**—The liquid is distilled up to a temperature of 200° C. at a pressure of 6 mm. of mercury.

## 4

phates), or by the hydrolysis of halides. It is also possible to prepare heavy poly-alcohols by the fixing of hypochlorous acid (or its homologues) and hydrolysis. The homologous oxides of ethylene oxide can also be obtained by the alkaline treatment of the chlorohydrins.

The treatment claimed hereinbefore for shale-oils can also be applied to certain fractions of the oil of distillation of lignite, which is relatively rich in unsaturated hydrocarbons.

The process of treatment, according to the invention, of shale-oils, can be illustrated by the following table, which is given by way of example, and which indicates the various operations to which the oil is subjected and which is followed by a small numerical table which also gives, by way of example, the characteristics of two fractions of oil obtained.

## Treatment

| No. of the fraction | Crude Gas Oil    |                           |                  |                          | Lubricating oil obtained |              |                 |                                                       |  |
|---------------------|------------------|---------------------------|------------------|--------------------------|--------------------------|--------------|-----------------|-------------------------------------------------------|--|
|                     | Density 15°/4°C. | Boiling point             | Density 15°/4°C. | Viscosity in centistokes |                          |              | Viscosity index | Yield by weight relatively to initial fraction of oil |  |
|                     |                  |                           |                  | at 35°                   | 30°                      | 100°         |                 |                                                       |  |
| 1.....              | 0.864            | °C.<br>203-282<br>252-323 | 0.9406           | 508<br>638               | 153<br>201               | 15.4<br>19.3 | -14<br>+19      | 18.4<br>16.5                                          |  |
| 2.....              | 0.880            |                           | 0.9407           |                          |                          |              |                 |                                                       |  |

The fixing of hydrochloric acid is particularly advantageous as regards the cost of production when this substance is obtained in the anhydrous state as a by-product of a condensation of aryl dichloride on the aromatic substances.

When these halogen derivatives are formed, polymerization or arylation can be obtained, not only with the catalysts already referred to, but with alkaline catalysts or alkaline alcoholates, such as sodium ethylate. The use of alkaline alcoholates enables OR groups (R being an organic radical) to be fixed on the molecules and, in the case of oil manufacture, the unctuousness of the lubricants obtained to be increased. If the operations are carried out on the halogen derivatives in such a manner as to obtain chlorinated oils, the unctuousness is also increased thereby.

By the co-polymerization of the halogen derivatives of the unsaturated hydrocarbons of shale-oil with fatty vegetable or animal halogen acids, esters or alcohols, it is possible to obtain viscous oils having a high viscosity index and of high unctuousness.

It is also possible to manufacture from the olefines of shale-oil all the usual olefine derivatives and in particular mono- and poly-alcohols, either by hydration (by hydrolysis of olefine sul-

50 be applied, separately or in combination, to shale-oils to make them into lubricating oils and other industrial petroleum products, include in particular the reacting of shale-oil with a suitable quantity of dihalo-alkyl, but this operation is only 55 considered in the foregoing as the complement of a prior arylation, for the purpose of which aromatic substances such as benzene or naphthalene or the like, were added to the oil.

Within the scope of the invention, it is also 60 possible to proceed in a reverse manner, that is to say react shale-oil with a dihalo-alkyl, without any prior addition, I have, in fact, discovered that shale-oil naturally contains a sufficient proportion of aromatic and possibly naphthenic hydrocarbons to react with dihalo-alkyl.

I have discovered, on the other hand, that this 65 operation can be effected just as well on the total oil as on a fraction, this being possible with or without the prior elimination of the bases and the phenols by acid and alkaline washing.

Finally, the dihalo-alkyls, that is to say the  $\alpha$ -dihalo-aliphatic hydrocarbons may be replaced by other dihalo-aliphatic hydrocarbons, in particular  $\omega$ -halogen hydrocarbons, such as di-75 chloro-1-3 propane, dichloro-1-4-butane,

The product obtained by this process has the characteristics of a lubricating oil which can be subjected to a distillation in vacuo to eliminate the comparatively light fractions and to adjust the viscosity of the residual oil which is the desired industrial product.

The following example shows the application of the process to a concrete case, it being of course understood that the invention is not limited to the data and conditions mentioned in this example.

*Example*

500 grams of shale-oil, previously treated with hydrochloric acid and with caustic soda in order to eliminate the bases and the phenols, are reacted with 100 grams of dichloro-ethane and 65 grams of anhydrous aluminum chloride.

The mixture is heated for 4 hours at boiling point in a flask provided with a reflux cooler; the temperature remains at 104-105° C.

The reaction is accompanied by the evolution of 20.14 grams of gaseous hydrochloric acid.

After hydrolysis and washing, the excess of dichloroethane is eliminated by distillation and 475 grams of raw treated oil are obtained, which represents a yield of 95 percent with respect to the oil involved.

The raw treated oil may be subjected to a distillation in vacuo in order to eliminate the relatively light fractions and to adjust the viscosity of the residual oil in accordance with the following table, which particularly shows a good viscosity index.

| Temperature<br>°C. | Pressure in<br>mm. Hg | Proportion of<br>distillate<br>relatively to<br>raw treated oil | Proportion of residual<br>oil relatively to— |                       | Viscosity of<br>residual oil<br>in c/stokes | Viscosity<br>index |
|--------------------|-----------------------|-----------------------------------------------------------------|----------------------------------------------|-----------------------|---------------------------------------------|--------------------|
|                    |                       |                                                                 | Raw<br>treated oil                           | Shale-oil<br>involved |                                             |                    |
| 96                 | 10                    | Percent                                                         | Percent                                      | Percent               | At<br>35° C.                                | 100° C             |
| 100                | 7                     | 11                                                              | 89                                           | 84.6                  | 34.6                                        | 4.95               |
| 100                | 7                     | 17.5                                                            | 82.5                                         | 78.5                  | 46.38                                       | 5.9                |
| 117                | 7                     | 27                                                              | 73                                           | 69.5                  | 87.05                                       | 8.66               |
| 150                | 7                     | 47                                                              | 53                                           | 50.5                  | 44                                          | 98                 |
| 160                | 7                     | 52                                                              | 48                                           | 45.6                  | 132                                         | 96.3               |

The present patent involves moreover improved methods relating to the application of the general process above described and which are intended to increase further the yield of viscous oil and decrease the consumption of catalyst.

In the first place, I have discovered that the treatment of the paraffin fractions of the crude oil does not produce any substantial increase in viscous oil, that it is therefore advantageous to remove these fractions prior to any treatment, and that it is thus possible to dispense with any deparaffining subsequent to the treatment, while obtaining oils having a suitable freezing point. This result is obtained by eliminating the heavy fractions of the oil, this elimination being more or less thorough according to whether a more or less low freezing point is desired for the finished oil.

With Autun shale oil, for instance, it has been found that it is necessary to reduce the oil to about 50% in order to obtain a freezing point of about +10° C., which in general is not sufficiently low for a lubricant. On the other hand, by only retaining about 37% of the oil, the freezing point is lowered to -10° C., this result being obtained without sacrificing in the slightest degree the increase of yield of viscous oil. This reduction amounts to fractionating the distillate at

175° C. at 20 mm. pressure, i. e. about 300° C. at atmospheric pressure.

The consumption of catalyst can be lowered if use is made of the tar from a first operation for catalysing one or more subsequent operations. I have discovered that this reuse is subject to several conditions:

1. Contrary to what might be expected, it is necessary for the fraction treated to be refined beforehand. Although the catalyst is capable of producing the refining effect, it is not advisable to allow this action to occur at the same time as the catalytic action. This prior refining is effected by the usual means, but preferably with dilute acid.

Furthermore, the treatment with earth, whether it forms the sole treatment or whether it follows the refining with acid, always has the effect of making the tars more flexible and more homogeneous, which contributes to make their re-use possible.

2. For the tar to remain utilizable, that is to say to retain a non-granular structure, it is necessary to adjust very accurately the stirring as a function of the temperature and of the duration of the reaction. There is an optimum adjustment for each operation, according to whether use is made of tar from 1, 2 . . . or *n* previous operations.

3. I have finally discovered, on the one hand, that the treatment of the non-oily distillates could further produce an appreciable yield of oil, and on the other hand that it is advantageous to prepare the catalyst, which is intended to act

on the crude oil, by starting to treat the non-oily distillates with said catalyst. The treatment of the distillates may increase by about 30 to 35% the yield of an operation or of the successive operations of treatment with tars.

On the other hand, the preparation of the catalyst by means of the distillates may enable the yield to be doubled, even including in said yield the gain obtained by treatment of the distillates.

An example, which is intended to make the invention clearly understood, is given hereinafter, without its being my intention to limit the invention to the numerical data chosen to illustrate the process.

An Autun shale oil is fractionated to 37.5%. Refining is effected three times with 2% of 10% hydrochloric acid at room temperature, the tars being separated out after each operation. The product is washed, then neutralized three times with 2% of 10% caustic soda. Decant, then after washing and further decantation, treat at a temperature of 75° C. with 5% of dried Aktisil earth. The necessary distillate for starting is obtained by treating a first charge in a reaction vessel holding 600 litres with a jacket for steam heating. The operation is effected at 80° C. in the presence

of 10% of  $\text{AlCl}_3$ ; the duration of the reaction is 2 hours.

The tars from this first operation serve for catalyzing a second operation at  $100^\circ \text{C}$ ., the duration of which is 3 hours. The tars from this second operation serve for catalyzing a third operation at  $100^\circ \text{C}$ ., the duration of which is  $3\frac{1}{2}$  hours.

Stirring is adjusted each time to the optimum speed which is predetermined by tests, in such a manner that the tars have a dry consistency after the second operation, and a granular consistency after the third operation (or after the last operation, if there are more than three).

The oily layer of each of the three operations is distilled. The three distillates, which represent about 65% of the total of the three charges, are not sufficiently viscous to possess lubricating properties and are mixed together. These distillates are subjected to a treatment with fresh aluminum chloride, the quantity of which is equal to 10% of the first charge. The operation is effected at  $80^\circ \text{C}$ ., for two hours. This operation produces an increase in the yield of viscous oil of about 7 to 10% relatively to the total of the three charges. The tars obtained by this operation serve for three fresh operations on crude oil in identical conditions to those hereinbefore specified. The mixed distillates of these three fresh operations serve for preparing with fresh aluminum chloride a fresh catalyst for three other operations on crude oil, and so forth.

The balance sheet of the yield works out as follows relatively to the crude oil:

|                                                              | Per cent | 35 |
|--------------------------------------------------------------|----------|----|
| Oil of viscosity 64 centistokes at $50^\circ \text{C}$ ----- | 35       |    |
| Oil of viscosity 45 centistokes at $50^\circ \text{C}$ ----- | 8        |    |
| Lamp oil -----                                               | 16       |    |
| Gas-oil -----                                                | 30       |    |
| Losses in refining -----                                     | 11       | 40 |
|                                                              | 100      |    |

The figure of three operations on crude oil per cycle is in no way limitative, this figure having been chosen only for the convenience of the explanation. I have even discovered that it is possible to recycle the distillate a second time and that, although the yield of oil from this second operation is not considerable, said operation produces on the other hand, interesting products.

The spirit of the invention is not altered by converting the process hereinbefore described into a continuous or a semi-continuous process.

I claim:

1. In a process of treating crude shale oil to produce a high grade lubricant therefrom, the steps of fractionating said crude shale oil to remove paraffin fractions therefrom, adding aromatic hydrocarbons to the residual portion of said oil, and then heating the oil in the presence of a Friedel and Crafts catalyst to simultaneously polymerize and arylate unsaturated constituents of said oil to convert them into compounds having improved lubricating properties.

2. In a process of treating crude shale oil to produce a high grade lubricant therefrom, the steps of treating the crude shale oil with hydrochloric acid to cause said acid to react with unsaturated constituents of said crude oil, simultaneously polymerizing and arylating the so treated oil in the presence of a Friedel and Crafts catalyst, mixing an alkyl dichloride with the polymerized and arylated oil, condensing said dichloride with aromatic constituents of said oil in the presence of a Friedel and Crafts catalyst to produce compounds having improved lubricating properties and hydrochloric acid, and using the hydrochloric acid produced in said condensation step for treating the crude oil in the first step above recited.

3. In a process of treating crude shale oil to produce a high grade of lubricant therefrom, the steps of fractionating said crude shale oil to remove paraffins therefrom, treating the fraction remaining after removal of said paraffins with hydrochloric acid to cause said acid to react with unsaturated constituents of said oil, simultaneously polymerizing and arylating the so treated oil in the presence of a Friedel and Crafts catalyst, mixing an alkyl dichloride with the polymerized and arylated oil, condensing said dichloride with aromatic constituents of said oil in the presence of a Friedel and Crafts catalyst to produce a product having improved lubricating properties and to produce hydrochloric acid, and using the hydrochloric acid produced in said condensation step for treating the crude oil in the second step above recited.

PAUL WOOG.

#### REFERENCES CITED

The following references are of record in the file of this patent:

#### UNITED STATES PATENTS

| Number    | Name                   | Date          |
|-----------|------------------------|---------------|
| 1,811,243 | Osmer -----            | June 23, 1931 |
| 1,954,972 | Young -----            | Apr. 17, 1934 |
| 2,051,612 | Loebel -----           | Aug. 18, 1936 |
| 2,080,701 | Day -----              | May 18, 1937  |
| 2,191,972 | Ocon -----             | Feb. 27, 1940 |
| 2,204,609 | Mikeska -----          | June 18, 1940 |
| 2,294,699 | Steffen -----          | Sept. 1, 1942 |
| 2,318,625 | Pier et al. -----      | May 11, 1943  |
| 2,318,719 | Schneider et al. ----- | May 11, 1943  |
| 2,365,751 | Drennan -----          | Dec. 26, 1944 |
| 2,398,908 | Miller -----           | Apr. 23, 1946 |
| 2,422,443 | Smith -----            | June 17, 1947 |
| 2,426,929 | Greensfelder -----     | Sept. 2, 1947 |

#### FOREIGN PATENTS

| Number  | Country       | Date          |
|---------|---------------|---------------|
| 713,149 | France -----  | Aug. 10, 1931 |
| 690,525 | Germany ----- | Apr. 29, 1940 |

#### OTHER REFERENCES

Dunstan et al., "The Science of Petroleum," vol. IV, Oxford University Press (1938), New York city, pages 3099 to 3103.